

1,032,973.

S. R., W. L. & J. B. WAGG.  
PROCESS OF SIZING PAPER.  
APPLICATION FILED JAN. 7, 1911.

Patented July 16, 1912.



Witnesses:

C. G. Hesler  
J. H. Geller

Inventors  
Solomon R. Wag<sup>g</sup>  
William L. Wag<sup>g</sup>  
James B. Wag<sup>g</sup>  
James L. Morris, Jr.  
atty.

# UNITED STATES PATENT OFFICE.

SOLOMON R. WAGG, WILLIAM L. WAGG, AND JAMES B. WAGG, OF APPLETON,  
WISCONSIN.

## PROCESS OF SIZING PAPER.

1,032,973.

Specification of Letters Patent. Patented July 16, 1912.

Application filed January 7, 1911. Serial No. 601,336.

To all whom it may concern:

Be it known that we, SOLOMON R. WAGG, WILLIAM L. WAGG, and JAMES B. WAGG, citizens of the United States, residing at 5 Appleton, in the county of Outagamie and State of Wisconsin, have invented new and useful Improvements in Processes of Sizing Paper, of which the following is a specification.

10 The present invention has reference to improvements in paper manufacture, and more especially in or relating to processes of sizing paper.

15 It comprehends, generally, a highly effective and economic sizing process which, when carried out in the manner hereinafter described, results in a very material increase in the tensile strength of the paper, and, at the same time, in a considerable decrease in cost by the avoidance of certain 20 expensive steps or treatments to which the web is ordinarily subjected, and the apparatus necessarily employed in connection therewith.

25 Briefly described, the process may be considered as subjecting the paper material to successive immersion in three separate baths of size: first, while in the form of wet pulp, it is subjected to a bath of resin size, where- 30 by the pulp is rendered capable of resisting ink and also of resisting moisture to the extent of permitting it to undergo the next treatment; second, the web formed subsequent to the application of the resin size is 35 passed through a solution of commercial acidulated starch, to further increase the tensile strength of the web; and, third, the starch sized web is immersed in a bath of animal glue, the previous coating of size 40 forming a cheap and solid foundation to which the glue size readily and permanently adheres. The process is essentially of a continuous nature, and the web is dried after each immersion and before being treated in 45 the succeeding bath, the particular character of the drying entering to a large degree into the invention and into its practicability and success.

50 In the accompanying drawing there is shown diagrammatically and partly in section the preferred embodiment of the apparatus in connection with which the process is worked. The receptacle or device in which the pulp sheet is subjected to the initial 55 bath of resin size is not, however, illus-

trated, since such receptacle or device may be of the ordinary type or of any preferred form.

In carrying out the process, the wet pulp is, as above stated, immersed in a bath of resin size. This bath is carefully prepared from what is known in the trade as resin "semi-soap" sizing, containing from 30% to 40% free resin. On being treated with hot water, a milk white solution is obtained 60 which is applied to the wet pulp just before the latter is formed into a web, the web-forming step being subsequently carried out in any suitable manner. The resin-impregnated web, designated in the drawing by the reference character *a*, is then led through the first drier *B*, the latter being here shown as comprising a series of steam-heated rolls *b* over and around which the web is passed. On leaving this drier, the 65 web is drawn through the size box or tub *C* containing the acidulated starch solution, and is then passed between the press-rolls *c*. During its passage through tub *C* the web 70 absorbs from 3% to 3½% of the starch, and its gain in tensile strength is from 30% to 45%. The web, coated and impregnated in this manner, is then subjected to a second thorough drying action by being passed around the steam-heated rolls *d* that compose the drier *D*, the coating of size being uninjured by the high heat of the rolls, which latter may, therefore, be rapidly revolved, and the sizing being, moreover, substantially invisible. From the second drier, 75 the web is led to the tub *E* containing the glue size and is drawn through the same and subsequently passed between the press-rolls *e*. The coating of glue size is applied, 80 as will be apparent, on top of the starch coating, and hence will fill up and seal any cracks therein that may have been produced during the second drying step, the glue adhering readily and effectively to the starch, 85 which latter constitutes a solid foundation or body for the same. Also, the application of the glue size to the previous coating of starch size has the effect of preventing much of the curling and crimping of the web that 90 would take place if the glue size were either applied directly to the web or mixed with the starch and the mixture then applied. The amount of glue size taken up by the web during its passage through tub *E* varies from 2½% to 3½%, and the total in- 95 100 105 110

crease in the tensile strength of the web from the time that it leaves the drier B will be found to vary from 90% to 100%. The glue-sized web, as has been proved from 5 actual experiments, cannot be dried by means of steam-heated rolls without great deterioration, owing to the inability of the size to resist the high temperature of said rolls. It becomes necessary, therefore, to 10 resort to a gradual or prolonged final drying at a comparatively low temperature, this final step, in practice, preferably taking place in a separate room from the room or rooms in which the treatments above described are carried out. To this end, the drier F is composed of a series of slowly 15 revolving skeleton drums *of* over and around which the web passes, the warm air in the room (at a temperature of from 70° to 20 90° F), being caused to circulate freely through the drums by fans or other suitable agitating devices, and being also directed by the same means against the web. From the final drier, the web passes to a 25 reel, (not shown), upon which it is wound in the ordinary manner.

The process above set forth is designed expressly for the production of high grade writing paper, and it may also be employed 30 with equal success in the manufacture of "cement bag" paper, the effect of the applications of the starch and glue size being to completely close the pores of the paper and to render the latter impervious to moisture and air. In that instance, the final drier may be of the same type as the driers B and D, though better results are obtained 35 when the skeleton drum drier is employed.

We claim as our invention:

40 1. A triple sizing process for paper material consisting in treating the material while in the form of wet pulp with a solution of resin size; immersing the subsequently-formed web in a bath of starch size; and

finally immersing the web thus treated in 45 a separate bath of glue size.

2. A triple sizing process for paper material consisting in treating the material while in the form of wet pulp with a solution of resin size; drying the subsequently-formed web; immersing the dried web in 50 a bath of starch size; drying the sized web; immersing said web in a separate bath of glue size; and finally drying the web thus treated. 55

3. A triple sizing process for paper material consisting in treating the material while in the form of wet pulp with a solution of resin size; drying the subsequently-formed web; immersing the dried web in 60 a bath of starch size; drying the sized web; immersing said web in a separate bath of glue size; and finally subjecting the web thus treated to a gradual drying by circulating a current of warm air therearound. 65

4. The process of sizing paper material which consists in treating the material while in the form of wet pulp with a solution of resin size; drying the subsequently-formed web; immersing the dried web in 70 a bath of starch size; drying the sized web; immersing said web in a separate bath of glue size; and finally in passing the web thus treated around a series of slowly revolving skeleton drums through which a 75 current of warm air continuously circulates to subject the web to a prolonged and gradual drying.

In testimony whereof we have hereunto 80 set our hands in presence of two subscribing witnesses.

SOLOMON R. WAGG.  
WILLIAM L. WAGG.  
JAMES B. WAGG.

Witnesses:

ORLANDO E. CLARK,  
THOS. B. REID.